

Patented Sept. 13, 1927.

1,642,485

# UNITED STATES PATENT OFFICE.

WILLIAM M. CHACE, OF DETROIT, MICHIGAN, ASSIGNOR TO W. M. CHACE VALVE COMPANY, A CORPORATION OF MICHIGAN.

## BIMETALLIC ELEMENT.

No Drawing.

Application filed July 6, 1925. Serial No. 41,887.

This invention relates to bimetallic elements, and the object is to secure a bimetallic element of high heat-resistant quality coupled with a comparatively high coefficient of expansion welded into a nickel-steel element of low coefficient of expansion.

I am aware of various compositions of metal used in bimetallic elements for instance brass and nickel-steel alloy and, while this element is practicable up to temperatures of about 450 degrees F., it becomes impracticable for use with higher temperatures. It is also necessary in a practical device for use under higher temperatures to provide a metal having a coefficient of expansion approximately equal to that of brass to secure an element readily responsive to temperature change. The element made of the two metals hereinafter described has this quality of ready responsiveness to temperature change except that it is slow to expand under temperatures below 200 degrees F., and is more readily responsive to higher degrees of temperatures. This also is an object of the invention to secure an element that is practically non-responsive or at least slow in responsiveness to temperatures below 200 degrees F. The bimetallic element herein described is useful wherever the element is subject to high temperatures as in making or breaking the electric circuit in an electric hand iron or in the controlling of the valve in oil refining systems for internal combustion engines and various other places and may have any desired form either as a disk as is used in the electric hand iron or as an elongated strip as is used in an ordinary thermostat depending upon the character of the apparatus with which it is used and the function it is to perform. With the electric hand iron the brass and iron bimetallic element is practically useless due to the fact that the brass loses its elasticity at about 450 degrees F., which I have termed its "critical temperature". This term as hereinafter used refers to the point beyond which the bimetallic element would become unreliable. With a structure in which brass forms one of the elements therefore it is impossible to utilize the same under temperature in excess of 450 degrees F., and in the electric hand iron the temperature thereof in use is approximately 600 degrees F. For this purpose sometimes metal known as "Monel metal" has been used as one of the

elements in conjunction with the nickel-steel alloy. The "critical temperature" of Monel metal, however, is about 600 degrees F., and therefore it is not of long life when used with an electric hand iron or other device wherein it is subject to such a temperature and furthermore requires too great a temperature change to cause movement of the element to the necessary extent.

One of the features of my improved bimetallic element is that its "critical temperature" is about 1200 degrees F., and is therefore useful in a great many places where previous elements of another type of metal is impracticable or not of long life.

My improved bimetallic element consists of a nickel-steel alloy in which the nickel content is from 36 to 42 per cent and which has a low coefficient of expansion and the other element which I have utilized has a coefficient of expansion approximately equal to that of brass—namely, about .070 inches per foot.

Preferably my composition consists of—

|           | Per cent. |
|-----------|-----------|
| Carbon    | .50       |
| Manganese | .70       |
| Silicon   | 1.75      |
| Chromium  | 8.00      |
| Nickel    | 22.00     |
| Copper    | 2.00      |
| Cobalt    | 1.00      |
| Iron      | 64.05     |

In making my bimetallic element I weld a bar of nickel-steel alloy and a bar of the above composition together and roll the same to the desired thinness. From this sheet is cut the element in the desired form either a disk or other shape as may be desired and depending upon the purpose for which it is to be used. This is the usual practice in the making of a bimetallic element. With my bimetallic element one member of which has a high coefficient of expansion formed of approximately the composition above stated and the other member of nickel-steel alloy I secure a bimetallic element as efficient at high temperatures as is the usual brass or Monel metal elements at lower temperatures; one which does not lose its elasticity at temperatures as high as 1200 degrees F., and therefore of long life when used or below such temperature, and further one that is very slow to expand at temperatures below

200 degrees F. My new element at temperatures above 200 degrees F., is readily responsive to heat and is perfectly adapted for use in such places as in controlling circuits 5 in an electric hand iron due to rapid responsiveness to temperatures around 600 degrees F., and which is affected readily by slight changes in temperature. In the usual Monel metal and steel alloy heretofore used with 10 an electric hand iron a change of approximately 10 degrees in temperature is required to effect making and breaking of circuit. With my composition the metal is responsive and will make and break the circuit within 15 a range of about 5 degrees F., it having a critical temperature of about 1200 degrees makes it very efficient for use with the electric hand iron and in other places where the element is subjected to temperature up to 20 1200 degrees F., and without loss of its elasticity.

A bimetallic element of the composition herein described will act approximately with equal rapidity to the previous brass and 25 nickel-steel elements or nickel-steel and Monel metal above mentioned and when used with an electric circuit in the form of a disk the flexing of the disk is so rapid under variations in temperature than in 30 breaking of the circuit no arcing occurs at the contacts.

I am aware of various compositions of metal used in bimetallic elements, and my invention consists not so much in the composition used as it does in the production of 35 a bimetallic element characterized by its heat resistant quality and rapid expansion under temperatures above 200 degrees F., and its slowness to expand under temperatures below 200 degrees F., combined 40 with a metal of much lower coefficient of expansion having a high percentage of nickel. The two elements welded together form a bimetallic element having the stated 45 qualities—namely, high heat resistant quality withstanding temperatures of practically 1200 degrees F., without impairing the elasticity of the element of high coefficient of expansion, is slow to respond to temperatures 50 below 200 degrees F., and above such temperatures expands and contracts as readily as the usual brass and steel elements.

Having thus described my invention what I claim and desire to secure by Letters Patent of the United States is—

1. A bimetallic element comprising two

metal elements fused together, each of said elements retaining its elasticity at temperatures as high as 1200 degrees F., one of said elements containing approximately forty per 60 cent nickel and characterized by having a low coefficient of expansion, and the other of said elements being of a composition in which iron predominates and characterized by its having a coefficient of expansion of 65 approximately .070 at temperatures above two hundred degrees F.

2. A bimetallic element having as one of the said elements a nickel-steel alloy in which the nickel content is not greater than forty-two per cent to which is welded a steel containing approximately the following composition—

|           |       |    |
|-----------|-------|----|
| Carbon    | .50   | 75 |
| Manganese | .70   |    |
| Silicon   | 1.75  |    |
| Chromium  | 8.00  |    |
| Nickel    | 22.00 |    |
| Copper    | 2.00  | 80 |
| Cobalt    | 1.00  |    |
| Iron      | 64.05 |    |

3. A bimetallic element having as one of its members a metal approximately of the following composition—

|           |       |    |
|-----------|-------|----|
| Carbon    | .50   |    |
| Manganese | .70   |    |
| Silicon   | 1.75  |    |
| Chromium  | 8.00  | 90 |
| Nickel    | 22.00 |    |
| Copper    | 2.00  |    |
| Cobalt    | 1.00  |    |
| Iron      | 64.05 |    |

and as the other member a metal of a lower 95 coefficient of expansion.

4. A bimetallic element consisting of two elements fused together, one of the elements being nickel steel alloy characterized by having a low coefficient of expansion and the other being of a composition of metals in which iron predominates and characterized by having a materially higher coefficient of expansion and capable of retaining its elasticity at a temperature as high as twelve 100 hundred degrees F., and being most rapidly expandible through a working range of from five hundred to seven hundred degrees F.

In testimony whereof, I sign this specification.

WILLIAM M. CHACE.